



US010053643B1

(12) **United States Patent**  
**Harvey**

(10) **Patent No.:** **US 10,053,643 B1**  
(45) **Date of Patent:** **Aug. 21, 2018**

(54) **FUELS AND LUBRICANTS FROM BISABOLINE**

(71) Applicant: **The United States of America, as Represented by the Secretary of the Navy**, Washington, DC (US)

(72) Inventor: **Benjamin G Harvey**, Ridgecrest, CA (US)

(73) Assignee: **The United States of America as Represented by the Secretary of the Navy**, Washington, DC (US)

(\*) Notice: Subject to any disclaimer, the term of this patent is extended or adjusted under 35 U.S.C. 154(b) by 75 days.

(21) Appl. No.: **14/919,114**

(22) Filed: **Oct. 21, 2015**

**Related U.S. Application Data**

(63) Continuation-in-part of application No. 13/676,541, filed on Nov. 14, 2012, now Pat. No. 9,994,498, and a continuation-in-part of application No. 14/314,305, filed on Jun. 25, 2014, now Pat. No. 9,493,717.

(60) Provisional application No. 61/562,681, filed on Nov. 22, 2011, provisional application No. 61/840,322, filed on Jun. 27, 2013.

(51) **Int. Cl.**

**C10L 10/10** (2006.01)  
**C10L 1/16** (2006.01)  
**C07C 5/03** (2006.01)  
**C07C 5/31** (2006.01)  
**C10L 1/08** (2006.01)  
**C10L 1/04** (2006.01)  
**C10L 10/12** (2006.01)  
**C10M 127/04** (2006.01)

(52) **U.S. Cl.**

CPC ..... **C10L 1/16** (2013.01); **C07C 5/03** (2013.01); **C07C 5/31** (2013.01); **C10L 1/04** (2013.01); **C10L 1/08** (2013.01); **C10L 10/10**

(2013.01); **C10L 10/12** (2013.01); **C10M 127/04** (2013.01); **C10L 1/1608** (2013.01); **C10L 2200/0469** (2013.01); **C10L 2270/026** (2013.01); **C10L 2270/04** (2013.01); **C10L 2290/24** (2013.01)

(58) **Field of Classification Search**

CPC ..... C10L 1/00; C10L 10/02  
See application file for complete search history.

(56)

**References Cited**

**U.S. PATENT DOCUMENTS**

|                 |         |                  |
|-----------------|---------|------------------|
| 7,846,222 B2    | 12/2010 | Renninger et al. |
| 8,703,454 B2    | 4/2014  | Schallk et al.   |
| 2008/0092829 A1 | 4/2008  | Renninger et al. |
| 2009/0020089 A1 | 1/2009  | Ryder et al.     |
| 2009/0020090 A1 | 1/2009  | Ryder et al.     |
| 2009/0272119 A1 | 11/2009 | Ryder            |
| 2009/0272352 A1 | 11/2009 | Ryder            |

(Continued)

**OTHER PUBLICATIONS**

U.S. Appl. No. 13/676,541, Benjamin Harvey.  
U.S. Appl. No. 13/604,115, Benjamin Harvey.

*Primary Examiner* — Ellen M McAvoy

*Assistant Examiner* — Ming Cheung Po

(74) *Attorney, Agent, or Firm* — Charlene A. Haley

(57)

**ABSTRACT**

A process for making high density fuels having the potential to increase the range and/or loiter time of Navy platforms. Derivation of these fuels from a sustainable source will decrease the carbon footprint of the Department of Defense (DoD) and reduce reliance on nonsustainable petroleum sources. Fuels derived from bisabolene can have volumetric net heats of combustion comparable to JP-10 and can be produced from biomass sugars.

**20 Claims, 3 Drawing Sheets**



(56)

**References Cited**

U.S. PATENT DOCUMENTS

2011/0056869 A1\* 3/2011 Novak ..... C10G 45/58  
208/49

2013/0298861 A1 11/2013 Lee et al.

\* cited by examiner



FIGURE 1



FIGURE 2



FIGURE 3

**1**  
**FUELS AND LUBRICANTS FROM  
 BISABOLINE**

**CROSS-REFERENCE TO RELATED  
 APPLICATIONS**

This is a continuation-in-part patent application of, claiming the benefit of, parent application Ser. No. 13/676,541 filed on Nov. 14, 2012, which claims benefit of patent application Ser. No. 61/562,681 filed on Nov. 22, 2011, and is a continuation-in-part patent application of, claiming benefit of patent application Ser. No. 14/314,305 filed on Jun. 25, 2014, which claims benefit of patent application Ser. No. 61/840,322 filed on Jun. 27, 2013, whereby the entire disclosures of which is incorporated hereby reference.

**STATEMENT REGARDING FEDERALLY  
 SPONSORED RESEARCH OR DEVELOPMENT**

The invention described herein may be manufactured and used by or for the government of the United States of America for governmental purposes without the payment of any royalties thereon or therefor. The Government and Contractor has certain rights in inventions made by the contractor and the Government employees while performing under the work statement of a Government funding agreement in Cooperative Research and Development Agreement (CRADA) #NCRADA-NAWCWDCL-14-255.

**FIELD OF THE INVENTION**

The invention generally relates to the conversion of sesquiterpenes to high density fuels. The invention relates to making high density fuels have the potential to increase the range and/or loiter time of Navy platforms.

**BRIEF DESCRIPTION OF THE DRAWINGS**

FIG. 1 is a block diagram illustrating the steps to produce high density biofuels from sesquiterpenes, according to embodiments of the invention.

FIG. 2 is a flow diagram illustrating the synthesis of high density fuels and lubricants from  $\alpha$ -bisabolene, according to embodiments of the invention.

FIG. 3 is a graph illustrating dynamic viscosity of alpha-bisabolene and bisabolane, according to embodiments of the invention.

It is to be understood that the foregoing general description and the following detailed description are exemplary and explanatory only and are not to be viewed as being restrictive of the invention, as claimed. Further advantages of this invention will be apparent after a review of the following detailed description of the disclosed embodiments, which are illustrated schematically in the accompanying drawings and in the appended claims.

**DETAILED DESCRIPTION OF EMBODIMENTS  
 OF THE INVENTION**

Embodiments of the invention generally relate to making high density fuels that have the potential to increase the range and/or loiter time of Navy platforms. Derivation of these fuels from a sustainable source will decrease the carbon footprint of the Department of Defense (DoD) and reduce reliance on nonsustainable petroleum sources. Fuels

derived from bisabolene can have volumetric net heats of combustion comparable to JP-10 and can be produced from biomass sugars.

The range of aircraft and weapon systems is largely dependent on the fuel used for propulsion. Fuels based on the monocyclic structure of bisabolane have volumetric net heats of combustion higher than conventional Navy jet fuel (JP-5) while maintaining an acceptable cetane number (>40). Further, bisabolene has three alkene groups which can be catalytically isomerized to generate fuels with net heats of combustion higher than JP-10. (>141,500 btu/gal) In addition, bisabolene can be generated from sustainable biomass sugars via fermentation. Use of these fuels will reduce net carbon emissions while improving the range and loiter time of a variety of Navy platforms.

1. alpha-bisabolene is generated via a fermentation process from substrates including biomass sugars and natural gas. Alternatively, alpha-bisabolene can be isolated from a renewable source, or generated by a metabolically engineered plant.

2. Bisabolene is catalytically isomerized to multicyclic hydrocarbons or bisabolene is dimerized to C30 hydrocarbons.

3. The product mixture is hydrogenated to yield a saturated mixture.

4. If desired the saturated mixture including cedrenes can be further isomerized to diamondoid structures.

5. Hydrogenated mixtures can be used directly as fuels or blended with other fuels to achieve desired properties.

30 Additives, including cetane enhancers can be added to the reduced sesquiterpenes to generate full performance jet or diesel fuels.

The following is a detailed description of some embodiments of the invention.

35 1. Alpha-bisabolene is generated from substrates including biomass sugars or natural gas via a fermentation process. Feedstocks can include cellulose, hemicellulose, glucose, sucrose, other reducing sugars, cellobiose, crude lignocellulosic materials, and lignin. Alternatively, mixtures of sesquiterpenes including bisabolenes can be isolated from plant extracts by steam distillation.

40 2. Bisabolenes are catalytically isomerized to multicyclic hydrocarbons with acid catalysts.

In embodiments the product mixture obtained via isomerization includes cedrenes. In embodiments the product mixture includes a complex mixture of multicyclic hydrocarbons. In embodiments the reaction can be allowed to go to completion or stopped at lower degrees of conversion to generate mixtures of bisabolenes and multicyclic sesquiterpenes. In embodiments the catalysts are heterogeneous acid catalysts. In embodiments, the bisabolene undergoes dimerization to yield multicyclic C30 hydrocarbons. In other embodiments, a mixture of multicyclic sesquiterpenes and C30 hydrocarbons are generated. The multicyclic hydrocarbons can then be separated by fractional distillation.

45 3. Antioxidants including phenolics are added to the unsaturated sesquiterpene mixture to increase the storage stability of the hydrocarbons. In a preferred embodiment, the sesquiterpene mixture is hydrogenated in the presence of a catalyst under a hydrogen atmosphere to obtain a saturated sesquiterpene mixture. A fuel mixture including only unsaturated bisabolene has the following properties: a net heat of combustion of 134, 150 btu/gal, a -20° C. viscosity of 10.5 cP, a 40° C. dynamic viscosity of 1.92 cP, and a density of 60 0.87 g/mL. A fuel mixture including only bisabolane has a net heat of combustion of 127,500 btu/gal, a -20° C. dynamic viscosity of 17.2 cP, a 40° C. dynamic viscosity of

2.1 cP, and a density of 0.814 g/mL. A fuel composed of hydrogenated cedrene has a net heat of combustion of ca. 142,000 btu/gal and a density of ca. 0.92 g/mL. Mixtures of bisabolane and cedrane have densities between 0.81 and 0.92 g/mL and NHOCs from 127-142,000 btu/gal. In embodiments saturated C15 hydrocarbons are separated from C30 dimers by fractional distillation after hydrogenation. The C30 hydrocarbons have applications as synthetic lubricants.

4. C15 mixtures including cedrenes or cedrane can be isomerized with a Lewis acid catalyst to yield hydrocarbons with diamondoid structures. In embodiments the diamondoid is 1-ethyl-3,5,7-trimethyladamantane.

5. Fuel mixtures including unsaturated sesquiterpene blends, saturated sesquiterpene blends, or diamondoid blends are combined with other renewable or petroleum-based fuels. In embodiments the sesquiterpene-derived fuels are blended with Jet-A, JP-8, JP-5, JP-10, RJ-4, F-76, commercial diesel fuel. In other embodiments, the sesquiterpene/pane fuels are blended with high cetane fuels derived via a Fischer-Tropsch process or Alcohol to-Jet (ATJ) process to generate fuels with cetane numbers in the range of 30-50. In other embodiments the sesquiterpene fuels are blended with nitrate esters or other cetane enhancers in low concentration to yield fuels with increased cetane numbers. In embodiments, further includes bisabolane blended with multicyclic sesquiterpanes or diamondoids to lower the viscosity of derivative fuels. In other embodiments, further includes bisabolane blended with multicyclic sesquiterpanes to improve the cetane number of the fuel in the range of 30-45.

Embodiments of the invention generally relate to methods for manufacturing jet and diesel fuels including, providing at least one  $\alpha$ -bisabolene A, a mixture of bisabolenes B, or a mixture of sesquiterpenes C including bisabolenes generated by metabolically engineered organisms from substrates including glucose, sucrose, fructose, other reducing sugars, cellobiose, cellulose, hemicellulose, lignocellulose, and methane, or isolated from plant material by solvent extraction or steam distillation, isomerizing the  $\alpha$ -bisabolene or bisabolene mixtures with a heterogeneous or homogenous acid catalyst to produce isomers, hydrogenating the isomers with at least one hydrogenation catalyst under hydrogen pressure and distilling the isomers to produce a first high density fuel and a higher molecular weight residue, or further isomerizing the isomers with a Lewis acid catalyst to generate a hydrocarbon mixture including adamantanes and distilling the adamantane mixture to produce a second high density fuel mixture and a higher molecular weight residue.

In embodiments, the isomer mixture includes multicyclic sesquiterpenes. In other embodiments, the isomer mixture includes cedrenes. In embodiments, the residue obtained after distillation of the first high density fuel is purified by vacuum distillation to yield a lubricant composed primarily of C30 hydrocarbons. In embodiments, the second high density fuel mixture having 1-ethyl-3,5,7-trimethyladamantane and other alkyladamantanes. In embodiments, the hydrogenating catalyst has at least one metal selected from the group consisting of Ni, Cu, Pd, Pt, Ru. In embodiments, the first acid catalyst is selected from the group consisting of at least one of perfluorinated sulfonic acid resins, cross-linked sulfonic acid resins, acid clays, zeolites, polyphosphoric acid, cation exchange resins, Lewis acid catalysts, metal oxides, supported Brønsted acid catalysts, mineral acids including  $H_2SO_4$  and  $H_3PO_4$ , and any mixtures thereof. In other embodiments, the Lewis acid catalyst is

selected from  $AlCl_3$ ,  $AlBr_3$ ,  $AlI_3$ , Lewis acidic ionic liquids,  $BF_3$ , gallium triflate, indium triflate, and other strong Lewis acids.

In embodiments, the first high density fuel has a density between 0.81 and 0.92 g/mL and a volumetric net heat of combustion from 124-142,000 btu/gal. In embodiments, the second high density fuel mixture has a density between about 0.88 and 0.94 g/mL and a volumetric net heat of combustion from 135-145,000 btu/gal. In embodiments, the first high density fuel or second high density fuel mixture has a cetane number between 30 and 42. In embodiments, the first high density fuel or second high density fuel mixture has a viscosity between about 10 and 60 cP at -20° C. In embodiments, the first high density fuel or second high density fuel mixture is blended with cetane enhancers including alkyl nitrates to generate fuels with cetane numbers >40.

In embodiments, the first high density fuel or second high density fuel mixture is blended with petroleum-based fuels including JP-10, RJ-4, JP-8, JP-5, F-76, Diesel #2, and Jet A. In embodiments, the first high density fuel or second high density fuel mixture is blended with a high cetane blendstock including fuels generated via a Fischer-Tropsch process, ethylene oligomerization, butene oligomerization, hexene oligomerization, to generate fuels with cetane numbers >40. In embodiments, the lubricant has a viscosity >20 cP at 40° C. In embodiments, the purified sesquiterpenes are combined with antioxidants including BHT and/or renewable phenols, and used as fuels without hydrogenation. Embodiments further include isomerizing the pure  $\alpha$ -bisabolene or bisabolene mixtures with at least one solvent. Another aspect of the invention generally relates to fuels produced by the methods herein.

FIG. 2. The catalytic conversion of  $\alpha$ -bisabolene to high density fuels and lubricants FIG. 3. The experimental dynamic viscosity of  $\alpha$ -bisabolene and bisabolane between -20 and 40° C.

The biosynthesis of farnesene and use as a standalone diesel/jet fuel or component of same is covered in the following USPTO applications: 20090272352, 20090272119, 20090020090, 20090020089, and 20080092829. Farnesane, the reduced form of farnesene, is a linear sesquiterpene of relatively low density (0.766 g/mL). U.S. Pat. No. 7,846,222 describes farnesane-based jet and diesel fuels. US patent application 20130298861 describes biosynthetic methods to generate bisabolene and discusses some fuels derived from bisabolene.

High density fuels have applications in a variety of Navy platforms including jet aircraft, ships, missiles, and UAVs. The fuels developed herein will help to meet Navy goals focused on the use of renewable and sustainable fuels while providing improved performance over conventional, petroleum-based fuels.

Embodiments of this invention describe the conversion of sesquiterpenes to high density fuels. The sesquiterpenes can be either extracted from plants or specifically produced by bioengineered organisms from waste biomass. This approach allows for the synthesis of high performance renewable fuels.

Embodiments of the invention detail processes for conversion of sesquiterpenes to high density fuel mixtures. Aspects of the process include hydrogenation of the sesquiterpenes to improve stability of the fuels as well as selective isomerization of the sesquiterpenes to improve density, net heat of combustion, low temperature viscosity, and cetane number. The isomerization process can be carried out with heterogeneous catalysts at moderate temperatures and

requires no solvent. Thus, embodiments of the invention provide a route for the sustainable production of renewable, ultra-performance fuels.

The general procedure for synthesizing high density sesquiterpene fuels is as follows:

1. A pure sesquiterpene or mixture of sesquiterpenes are either extracted from plant sources (e.g. clove oil) or

2. a) A biomass source (including lignocellulosic, cellulosic, or hemicellulosic feedstocks) is hydrolyzed to produce a sugar solution

b) The sugar solution is fermented to a sesquiterpene or mixture of sesquiterpenes by a bioengineered organism.

3. The hydrocarbons are purified by solvent extraction, pervaporation, membrane separation, or distillation.

4. Pure sesquiterpenes or mixtures are then:

a) Directly hydrogenated and distilled to yield a liquid fuel or

b) Isomerized with heterogeneous acidic catalysts to produce a pure compound or complex mixture of hydrocarbons which is then hydrogenated and distilled to yield a liquid fuel.

Process:

1. A pure sesquiterpene or mixture of sesquiterpenes is isolated from a plant source. This can be accomplished by steam distillation, solvent extraction, or pyrolysis, among other techniques.

2a. In an alternate approach, biomass can be hydrolyzed to produce a sugar solution. This step can be accomplished by physical, chemical, or enzymatic methods, or any combination thereof.

2b. The sugar solution is used as a food source for bioengineered organisms that produce sesquiterpenes in either a batch or continuous mode.

3. Regardless of the source, the sesquiterpenes can be upgraded through techniques including fractional distillation, chemical treatments, and extractions to produce a suitably pure hydrocarbon feedstock composed of either a single sesquiterpene or complex mixture of sesquiterpenes. In the case of the biosynthesized sesquiterpenes (2b), the major impurity is water which can be effectively removed by both membrane separation techniques as well as by distillation.

4a) Sesquiterpenes are directly hydrogenated to produce a high density fuel. Catalysts based on Ni, Pd, Pt, Cu, and Ru can be utilized under moderate hydrogen pressures.

4b) To improve specific fuel properties such as viscosity, net heat of combustion, density, and cetane number, sesquiterpenes can be readily isomerized with heterogeneous acid catalysts including, but not limited to: Naftion, Amberlyst, Montmorillonite K-10, zeolites and supported polyphosphoric acid. Sesquiterpenes can also be effectively isomerized with Lewis acids and mineral acids. After isomerization, these sesquiterpenes can be hydrogenated as in 4a. Pure sesquiterpenes or defined mixtures of sesquiterpenes can be isolated by fractional distillation to generate fuels with specific properties. FIG. 1 is a block diagram overview showing the steps of the embodiments of the invention therein.

Example 1 (high catalyst loading). 50 mL of caryophyllene (technical grade) is combined with 500 mg of Nafion SAC-13 in a flask. The mixture is vigorously stirred and heated to 100° C. overnight. The pale yellow solution is decanted, hydrogenated at 50 psig H<sub>2</sub> with 50 mg PtO<sub>2</sub> as catalyst. The resulting mixture is filtered and vacuum distilled to yield a colorless fuel mixture including saturated

hydrocarbons derived from seven main isomers including  $\alpha$ -neoclovene, clovene, and  $\alpha$ -panasinsene (see Schematic 1).

Schematic 1. Products resulting from the acid-catalyzed isomerization of  $\beta$ -caryophyllene. Numbers under the structures represent the weight percentage of each molecule. The first number results from low catalyst loading, while the number in parentheses results from high catalyst loading as described in the process.

10



Example 2 (low catalyst loading). 500 mL of caryophyllene is combined with 2 g of Nation SAC-13 in a flask and subjected to the same conditions as in Example 1. A significantly different product distribution results (see Schematic 1).

Example 3. 175 mL of valencene (Scheme 3) biosynthesized from sucrose is hydrogenated at 50 psig 1H<sub>2</sub> with 100 mg PtO<sub>2</sub> as catalyst. After hydrogenation the catalyst floculates and the catalyst is separated by decantation. The properties of this fuel mixture are listed in Table 1.

Example 4. 175 mL of prennaspirodiene (Scheme 3) biosynthesized from sucrose is hydrogenated as in Example 3. The properties are listed in Table 1.

Example 5. 175 mL of commercial caryophyllene (technical grade) is hydrogenated as in Example 3. The properties are listed in Table 1.

Example 6. 5 g of valencene biosynthesized from sucrose are combined with 0.1 g of Nafion SAC-3 and the mixture is stirred and heated to 100° C. for 16 h. The solution is decanted to yield a mixture of isomers.

Example 7. 5 g of prennaspirodiene biosynthesized from sucrose is isomerized as described in Example 6.

TABLE 1

| Key Properties of Sesquiterpene Fuels.         |                |                |                        |                         |                     |                    |
|------------------------------------------------|----------------|----------------|------------------------|-------------------------|---------------------|--------------------|
| Table 1. Key Properties of Sesquiterpene Fuels |                |                |                        |                         |                     |                    |
| Sesquiterpene                                  | Density (g/mL) | NHOC (btu/gal) | 40° C. Viscosity (cSt) | -20° C. Viscosity (cSt) | Ignition Delay (ms) | Derived Cetane No. |
| Valencane                                      | 0.879          | 135,386        | 4.417                  | 50.24                   | 10,562              | 23.26              |
| Caryophyllane                                  | 0.85           | 132,790        | 4,067                  | 60.47                   | 9.75                | 24.52              |
| Premnaspriodiane                               | 0.882          | 135,564        | 3.812                  | 42.91                   | 7.779               | 28.65              |
| HDCL-8                                         | 0.90           | 137,800        | 53.58                  | NM                      | 13.173              | 20.23              |
| HDCL-9                                         | 0.90           | 137,100        | 5.07                   | 61.96                   | 6,549               | 32.53              |
| HDCL-10                                        | 0.92           | 140,900        | NM                     | NM                      | NM                  | NM                 |

## Note:

HDCL-8 is the fuel generated from caryophyllene with high catalyst loading, HDCL-9 is the fuel generated with low catalyst loading. The density and net heat of combustion of HDCL-10 has been calculated based on a distillate cut including primarily high-density components (i.e. clovane/neoclovane and assuming a density of 0.92 g/mL).

Scheme 2. Isomerization of caryophyllene with heterogeneous acid catalyst.



Scheme 3. Structures of valencene and premnaspriodiene.



Embodiments of the invention generally relate to methods for manufacturing jet and diesel fuels including, providing pure and/or mixed sesquiterpenes isolated from plant extracts and/or biosynthesized from biomass, purifying the pure and/or mixed sesquiterpenes to produce single components or mixtures of sesquiterpenes, converting the single component or mixed sesquiterpenes by either, directly hydrogenating the single component or mixed sesquiterpenes with at least one hydrogenation catalyst under hydrogen pressure, or isomerizing either with or without a solvent, the single component or mixed sesquiterpenes with at least one heterogeneous acid catalyst to produce isomers and

hydrogenating the isomers with at least one hydrogenation catalyst under hydrogen pressure, and distilling either the 20 hydrogenated single component or mixed sesquiterpenes or the hydrogenated isomers to produce high density fuels.

Another aspect of the invention generally relates to the production and blends of fuels. In embodiments, the pure and/or mixed sesquiterpenes are selected from the group consisting of valencene, premnaspriodiene, caryophyllene, humulene, clovane, neoclovane, panasinsene, thujopsene, longifolene, cubebene, zizaene, santalene, longipinene, isomers of the above sesquiterpenes, other cyclic terpenes, and any mixtures thereof. In embodiments, the single component or mixed sesquiterpenes are selected from the group consisting of caryophyllene, valencene, premnaspriodiene, or any mixture thereof. In embodiments, the isomers are at least one isomer selected from the group consisting of 30  $\alpha$ -neoclovane, clovane, or any mixture thereof. In embodiments, the hydrogenating catalyst having at least one metal selected from the group consisting of Ni, Cu, Pd, Pt,  $\text{PtO}_2$ , Ru and the reaction is conducted without a solvent.

In embodiments, the heterogeneous acid catalyst are 40 selected from the group consisting of at least one of Nafion (perfluorinated sulfonic acid resins), Amberlyst (cross-linked sulfonic acid resins), Montmorillonite K-10, zeolites, polyphosphoric acids, cation exchange resins, Lewis acid catalysts, supported Bronsted acid catalysts, mineral acids 45 including  $\text{H}_2\text{SO}_4$  and  $\text{H}_3\text{PO}_4$ , and any mixtures thereof. In embodiments, the plant extracts are selected from the group consisting of clove oil or any essential oil having significant quantities of cyclic sesquiterpenes, and mixtures of said oils. In embodiments, the biomass includes at least one of 50 sucrose, glucose, fructose, cellobiose, other reducing sugars, cellulose, and hemicelluloses in any proportion.

Another aspect of the invention generally relate to methods for manufacturing jet and diesel fuels including, providing pure and/or mixed sesquiterpenes isolated from plant 55 extracts and/or biosynthesized from biomass, purifying the pure and/or mixed sesquiterpenes to produce single components or mixtures of sesquiterpenes producing a first set of fuels, or converting the single component or mixed sesquiterpenes by isomerizing either with or without a solvent, the 60 single component or mixed sesquiterpenes with at least one heterogeneous acid catalyst to produce isomers, and distilling the isomers producing a second set of fuels. All blends of fuels are incorporated into all aspects of the invention.

Yet other aspects of the invention generally relate to a first 65 set of fuels produced from the methods above. Still yet other aspects of the invention generally relate to a second set of fuels produced from the methods above.

In embodiments, the fuels are pure sesquiterpanes or prepared by selective fractional distillation of sesquiterpane mixtures (density >0.90 g/mL, NHOC>137,000 btu/gal). In other embodiments, the fuels are pure sesquiterpanes or generated by selective fractional distillation of sesquiterpane mixtures (cetane number >30). In yet other embodiments, the fuels are generated by blending sesquiterpane mixtures with known cetane enhancers or antioxidants for fuels. In embodiments, the fuels generated by blending sesquiterpene fuels with petroleum-based fuels including JP-10, RJ-4, JP-8, JP-5, F-76, Diesel #2, Jet A, and any renewable fuel.

In embodiments, the high density missile/turbine fuels are blends of cyclic sesquiterpanes with JP-10 in a desired proportion. In embodiments, the high density jet fuels are blends of cyclic sesquiterpanes with jet fuels including JP-5, JP-8, and Jet A. In embodiments, the high density diesel fuels are blends of cyclic sesquiterpanes with petroleum-derived diesel fuel. In embodiments, the high density jet/diesel fuels are blends of cyclic sesquiterpanes with fuels generated by ethylene oligomerization. In embodiments, the high density jet/diesel fuels are blends of cyclic sesquiterpanes with fuels generated by butene oligomerization. In embodiments, the high density jet/diesel fuels are blends of cyclic sesquiterpanes with fuels generated by hexene oligomerization. In embodiments, the high density jet/diesel fuels are blends of cyclic sesquiterpanes with diesel fuels produced from natural gas.

Where a range of values is provided, it is understood that each intervening value, to the tenth of the unit of the lower limit unless the context clearly dictates otherwise, between the upper and lower limits of that range is also specifically disclosed. Each smaller range between any stated value or intervening value in a stated range and any other stated or intervening value in that stated range is encompassed within the invention. The upper and lower limits of these smaller ranges may independently be included or excluded in the range, and each range where either, neither or both limits are included in the smaller ranges is also encompassed within the invention, subject to any specifically excluded limit in the stated range. Where the stated range includes one or both of the limits, ranges excluding either or both of those included limits are also included in the invention.

While the invention has been described, disclosed, illustrated and shown in various terms of certain embodiments or modifications which it has presumed in practice, the scope of the invention is not intended to be, nor should it be deemed to be, limited thereby and such other modifications or embodiments as may be suggested by the teachings herein are particularly reserved especially as they fall within the breadth and scope of the claims here appended.

What is claimed is:

1. A method for manufacturing jet and diesel fuels, consisting of:

providing at least one  $\alpha$ -bisabolene A, a mixture of bisabolenes B, or a mixture of sesquiterpenes C including bisabolenes generated by metabolically engineered organisms from substrates including glucose, sucrose, fructose, other reducing sugars, cellobiose, cellulose, hemicellulose, lignocellulose, lignin, and methane, or isolated from plant material by solvent extraction or steam distillation; isomerizing said  $\alpha$ -bisabolene or bisabolene mixtures with a heterogeneous or homogenous acid catalyst to produce isomers; and hydrogenating said isomers with at least one hydrogenation catalyst under hydrogen pressure and distilling said

isomers to produce a first high density fuel and a higher molecular weight residue; or further treating said isomers with a Lewis acid catalyst to generate a hydrocarbon mixture including alkyladamantanes and distilling the alkyladamantane mixture to produce a second high density fuel mixture and a higher molecular weight residue.

2. The method according to claim 1, wherein the isomer mixture having multicyclic sesquiterpenes.

3. The method according to claim 1, wherein the isomer mixture having cedrenes.

4. The method according to claim 1, wherein said residue obtained after distillation of the first high density fuel is purified by vacuum distillation to yield a lubricant composed primarily of C30 hydrocarbons.

5. The method according to claim 1, wherein the said second high density fuel mixture having 1-ethyl-3,5,7-trimethyladamantane and other alkyladamantanes.

6. The method according to claim 1, wherein said hydrogenating catalyst has at least one metal selected from the group consisting of Ni, Cu, Pd, Pt, Ru.

7. The method according to claim 1, wherein the first acid catalyst is selected from the group consisting of at least one of perfluorinated sulfonic acid resins, cross-linked sulfonic acid resins, acid clays, zeolites, polyphosphoric acid, cation exchange resins, Lewis acid catalysts, metal oxides, supported Brønsted acid catalysts, mineral acids including  $H_2SO_4$  and  $H_3PO_4$ , and any mixtures thereof.

8. The method according to claim 1, wherein the Lewis acid catalyst is selected from  $AlCl_3$ ,  $AlBr_3$ ,  $AlI_3$ , Lewis acidic ionic liquids,  $BF_3$ , gallium triflate, indium triflate, and other strong Lewis acids.

9. The method according to claim 1, wherein said first high density fuel has a density between 0.81 and 0.92 g/mL and a volumetric net heat of combustion from 124-142,000 btu/gal.

10. The method according to claim 1, wherein said second high density fuel mixture has a density between about 0.88 and 0.94 g/mL and a volumetric net heat of combustion from 135-145,000 btu/gal.

11. The method according to claim 1, wherein said first high density fuel or second high density fuel mixture has a cetane number between 30 and 42.

12. The method according to claim 1, wherein said first high density fuel or second high density fuel mixture has a viscosity between about 10 and 60 cP at -20° C.

13. The method according to claim 1, wherein said first high density fuel or second high density fuel mixture is blended with cetane enhancers including alkyl nitrates to generate fuels with cetane numbers >40.

14. The method according to claim 1, wherein said first high density fuel or second high density fuel mixture is blended with petroleum-based fuels including JP-10, RJ-4, JP-8, JP-5, F-76, Diesel #2, and Jet A.

15. The method according to claim 1, wherein said first high density fuel or second high density fuel mixture is blended with a high cetane blendstock including fuels generated via a Fischer-Tropsch process, ethylene oligomerization, butene oligomerization, hexene oligomerization, to generate fuels with cetane numbers >40.

16. The method according to claim 4, wherein said lubricant has a viscosity >20 cP at 40° C.

17. The method according to claim 1, wherein said purified sesquiterpenes are combined with antioxidants including BHT and/or renewable phenols, and used as fuels without hydrogenation.

**18.** The method according to claim 1, further comprising isomerizing said pure  $\alpha$ -bisabolene or bisabolene with at least one solvent.

**19.** The method according to claim 1, further comprising bisabolane blended with multicyclic sesquiterpanes or dia- 5 monoids to lower the viscosity of derivative fuels.

**20.** The method according to claim 1, further comprising bisabolane blended with multicyclic sesquiterpanes to improve the cetane number of the fuel in the range of 30-45.

\* \* \* \* \*

10